

E. F. GOLTRA.  
PROCESS FOR CLEANING IRON ORES.  
APPLICATION FILED OCT. 18, 1909.

961,121.

Patented June 14, 1910



## Witnesses

J. G. Linkel  
J. H. Brumunga.

Inventor

Edward F. Galts

By

Foster, Freeman, Watson & Cie

Attorneys

# UNITED STATES PATENT OFFICE.

EDWARD F. GOLTRA, OF ST. LOUIS, MISSOURI.

## PROCESS FOR CLEANING IRON ORES.

961,121.

Specification of Letters Patent. Patented June 14, 1910.

Application filed October 18, 1909. Serial No. 523,091.

*To all whom it may concern:*

Be it known that I, EDWARD F. GOLTRA, a citizen of the United States, and resident of St. Louis, in the State of Missouri, have invented certain new and useful Improvements in Processes for Cleaning Iron Ores, of which the following is a specification.

This invention relates to a process for cleaning iron ores and for preparing the same for the subsequent operations.

Some iron ores, as brown hematite, contain a large percentage of clay and sometimes silica as a gangue, and this gangue must be separated from the ore before it can be used in a blast furnace.

In my co-pending application, Serial No. 536,403, filed January 4, 1910, a process is described whereby iron ore is cleaned of its gangue by a blast.

The objects of this invention are to refine the process broadly described and claimed in the above application so as to render it continuous.

This invention generally stated consists in the operations as hereinafter fully described and claimed.

The apparatus preferably consists of a runway upon which the ore is thrown. The ore on the runway is subjected to a strong blast so as to dry the gangue and render the earthy, the silicious and any other gangue easily separable from the ore. The ore is tumbled to shake loose the gangue from the ore, and the gangue is removed by the blast.

The runway is preferably in the form of a long inclined tube or drum, which is rotated about its longitudinal axis, and a hopper is located at one end of the drum for discharging the ore into the same. The ore in its passage downwardly is heated to dry out the ore and render the gangue brittle and easily separable from the ore, and the rotation of the drum will tumble and rattle the ore as it dries and cause the gangue to be shaken loose from the ore and pulverized by the tumbling action. The strong blast sweeps, cleans and washes the gangue from the ore and this gangue is withdrawn from the drum by the blast while the cleaned ore passes along the drum to the discharge end.

The ore as mined must be dried slowly especially if it contains much clay as a gangue since a rapid heating would cause this clay to be baked hard and burned to a brick and thus it would be impossible or ex-

ceedingly difficult to thereafter loosen it from the ore. For this purpose the hot blast enters the drum at the lower end, that is at the discharge end, and when it strikes the fresh ore admitted from the hopper this hot blast is cooled down enough so that its temperature is sufficiently low to prevent the hard baking and burning of the gangue.

In the drawing the figure is a view showing one form of apparatus whereby the process may be carried out.

Referring to the drawing, 10 designates a runway in the form of a tube or drum provided with a number of rings 11, 11, resting on a number of sets of anti-friction rollers 12, 12. The ends of the drum extend into stationary heads 13, 14 which are bolted to a suitable frame-work, and the hopper 15 on head 13 discharges into the drum. A suction fan 16 is connected to the head 14 and is driven by a suitable motor so as to create a strong blast in and through the drum 10. A burner 17 extends through the head 13 so as to heat the blast. This burner may be an ordinary oil burner provided with an air blast. The head 13 is further provided with an air hole 21, or air holes, so as to allow the blast to enter near the burner and be heated thereby. The head is further provided with a discharge or outlet 18 for the cleaned ore. The drum is inclined from the inlet to the discharge end and is rotated by a driving pinion 19 engaging a gear 20 on the drum. The drum is lined with a suitable refractory lining 22.

The ore as mined is crushed so as to reduce it to workable form. It is not necessary to pulverize it, but it is sufficient if it can pass through a two or two and one-half inch mesh. This crushed ore is placed in the hopper 15 and is discharged into the drum 10. The burner 17 furnishes the necessary heat and the temperature will be the greatest at the lower end of the drum, but at the upper end this temperature will be considerably reduced, so that the fresh wet ore will not be heated to a sufficient degree so as to hard bake the gangue. As the ore moves downwardly it will be tumbled and thrown around so as to knock loose all of the gangue which clings to it, this gangue becoming more and more heated and more and more loose, dried and pulverized as it proceeds toward the lower end of the drum. The ore is cleaned and washed of its gangue by the

blast passing through the drum, the gangue being drawn off by the strong blast which is created by the suction fan 16. The drum is made long enough and the speed of rotation 5 is governed so that at the time when the ore reaches the discharge 18 practically all of the gangue has been dried out and rendered separable, shaken off of the ore and drawn off by the blast. Since the temperature will 10 gradually increase from the upper to the lower end of the drum, the ore is gradually dried and thus the gangue is rendered very brittle, and due to this gradual increase, the gangue on the ore as it is admitted will not 15 be subjected to the high temperature as would be the case if the burner 17 were placed at the upper end of the drum.

In the form of the invention shown in the figure the heat is generated by a burner 17. 20 It is, however, advantageous in some instances to generate this heat by passing a hot blast directly through the aperture 21 in the head 13, and into the lower end of the drum 10. It is also obvious that the ore may be 25 heated in any other suitable manner, therefore, it is to be understood that this invention is not to be limited to the specific means for heating the ore. Where a hot blast is 30 directly used for furnishing the heat the fan 16 may be dispensed with if desired.

It will be noted that the blast is passed through and above the ore while it is agitated. The rotation of the drum will cause the ore to rise with the sides of the drum 35 and fall through the blast passing through the drum. In this way the strong blast sweeps the pulverized gangue clinging to and surrounding the ore with it, allowing the cleaned ore to pass down the drum to the 40 discharge 18. The blast seeks out the gangue in the crevices and around the ore and carries it away with it. It will be remembered that the pieces of ore are comparatively large and heavy and therefore in 45 their tumbling motion practically all the gangue will be knocked off and pulverized.

The length of the drum, its diameter, its 50 incline, the speed of rotation and the temperatures will vary with different ores and with their condition as to dampness, the amount of clay in them, etc. As a practical case, where an oil burner is used the temperature at the lower end of the drum will be 2000° F. or over, while the temperature 55 at the upper end will be 300° to 400° F. In all cases however, the process is so regulated that the gangue will be dried and rendered separable, shaken loose, and separated, the temperatures being controlled so that the 60 gangue will be thoroughly dried and still dried gradually enough so that it will not become hard baked. Another important result obtained is that the moisture in the ore is driven off during this process, leaving the 65 cleaned ore in a dry porous condition. Thus

the amount of heat necessary in the other operations is materially reduced.

It is obvious that various changes may be made without departing from this invention, and it is therefore to be understood 70 that this invention is not to be limited to the specific arrangements shown and described.

The broad process is broadly claimed in my co-pending application Serial No. 75 536,403, referred to.

Having thus described the invention, what is claimed is:

1. The herein described process of treating iron ores containing moist clay, etc., as 80 a gangue, which consists in heating the ore and its gangue at a temperature and for a period sufficient to drive off the moisture and to render the gangue easily separable from the ore, tumbling the ore and its 85 gangue during the heating operation to shake loose the gangue from the ore, and to pulverize the gangue by said tumbling action, and subjecting the ore and its gangue during the heating and tumbling operation 90 to a strong gaseous blast which sweeps, cleans and removes the gangue from the ore.

2. The herein described process of treating iron ores containing moist clay, etc., as 95 a gangue, which consists in subjecting the ore and gangue to a strong hot gaseous blast at a temperature and for a period sufficient to drive off the moisture and render the gangue easily separable from the ore, tumbling the ore and its gangue during the heating operation to shake loose the gangue from the ore and to pulverize the gangue by 100 said tumbling action, and sweeping, cleaning, and removing the gangue from the ore 105 by said blast during the heating and tumbling operation, the blast being applied to strike the drier portions of the ore and gangue before the damper portions to gradually heat the gangue.

3. The herein described process of treating iron ores containing moist clay, etc., as 110 a gangue, which consists in passing the ore and its gangue along a runway, passing a strong hot gaseous blast along said runway 115 from the discharge to the admission end so as to gradually heat and dry the gangue and render it easily separable from the ore, tumbling the ore and its gangue in their passage along the runway to shake loose 120 the gangue from the ore, and to pulverize the gangue by said tumbling action, and sweeping, cleaning, and removing the gangue from the ore by said blast.

In testimony whereof I affix my signature in presence of two witnesses.

EDWARD F. GOLTRA.

Witnesses:

J. H. BRUNINGA,  
WALTER E. PAUL.